

## UNITED STATES PATENT OFFICE

2,609,295

PROCESS FOR DISCONTINUOUSLY PHYSI-  
CALLY DEVELOPING LATENT PHOTO-  
GRAPHIC IMAGES

Roelof Jan Hendrik Alink, Cornelis Johannes Dippel, and Harke Jan Houtman, Eindhoven, Netherlands, assignors to Hartford National Bank and Trust Company, Hartford, Conn., as trustee

No Drawing. Application October 8, 1948, Serial No. 53,605. In the Netherlands October 27, 1947

6 Claims. (Cl. 95—6)

1

The invention relates to a method of producing contrasts, consisting of metal, in photographic material by physical development of latent images in sensitized, lyophilic supports, the term "physical development" being understood to mean a method of developing according to which, prior to development, all the metal required for building up the contrast does not yet occupy its position in the contrast as an ion or as a compound and the term "latent image" being understood to mean the image which is produced by mere exposure of the photographic material before external measures are taken to intensify this image; in some cases the said image may already be visible.

This physical development is carried out with the use of a metal compound adapted to be reduced to metal in an aqueous solution, such as a salt of mercury, silver, gold or platinum, and of a reducing agent. By way of example may be mentioned here the development to form a silver image of a latent mercury image produced by exposure of a light-sensitive system consisting of a diazonium compound and a mercurous salt (British patent specification 439,005).

The physical developers referred to are unstable systems. Even when not in use, they deteriorate rapidly with the separation of metal; they are therefore uneconomical in practical use and contaminate and in addition metal is liable to be deposited during the developing process even at unexposed areas of the light-sensitive layer, which may result in fogging.

These difficulties are such that hitherto such a physical development, without the laboratory, has never been carried out on an industrial scale. The methods hitherto suggested invariably amount to bringing the photographic material into contact with a supply of fresh developer, which has become unserviceable at the end of the development, considerable contamination generally occurring due to metal being separated out of the solution. It is true that it is possible to produce developers which are comparatively stable according to the standards applying for physical development, but the stabilisation also results in a deceleration of the development, so that for most purposes the latter proceeds excessively slowly, whilst at the same time the stabilized developer can only be used on one occasion.

It should be noted that technical use of physical development is attractive. For definite kinds of photographic material (vide, for example, the above-mentioned British patent specification 439,005) treatment is even confined

2

thereto. In other cases physical development is desired from considerations of the quality of the image, for example, in view of the high resolving power which can be obtained therewith. However, in the technical use of physical development the problem arises as to how large quantities of photographic material are to be readily worked up and how waste of chemicals is to be avoided as far as possible. For this purpose efforts may be made, for example, to carry out physical development as a continuous process or, as an alternative, to solve the problem, while maintaining the discontinuous nature of physical development. For strip-like photographic material such an effort resulted in the method described in the British patent specification 545,901, according to which a large length of such material is wound on a drum and is treated with a restricted quantity of physical developer. The present invention provides a solution of the same problem, which solution permits of satisfying a completely different need out of practice, that is to say physical development of large numbers of sheets of photographic material. It often occurs, for example, that photostat copies of printed texts are required to be made. Attempts could be made to design a continuously operating machine for this purpose. However, such a machine requires regular supply of photographic material and when in use presents the difficulties attendant on the use of continuous physical development, that is to say the problem of avoiding soiling and that of refreshing the developer. On the other hand discontinuous physical development is unserviceable here without further expedients: fresh developer is required to be made at intervals, considerable supervision is needed, the production is excessively small and the waste of chemicals in the exhausted developer is excessive. The invention has for its object to obviate these latter difficulties.

According to the invention, lyophilic photographic material in the form of a pile of sheets is developed in a stable physical slow-action developer which contains not more than approximately three times the quantity of metal salt which just suffices for building up the contrasts. For measuring an exactly suitable quantity of the metal salt it should be noted in the case of silver images that for the development of 1 square metre of photographic material so as to produce a mean blackening in transparency of 1 approximately 2 gms. of silver nitrate suffice. A "stable" physical developer is understood to mean here a physical developer in which 15 minutes after its

preparation, that is to say after mixing the solution of the metal salt and the solution of the reduction agent, visible separation of metal in the liquid has not yet occurred. The times of development in such stable physical developers are generally also at least 15 minutes. Long times of development have the advantage that the duration of development is not particularly important so that less supervision is required during development. If moreover use is not made in such a developer of considerably more metal salt than is sufficient for building up the contrasts, it is only this small excess of metal salt which may result in deposition of metal at undue, that is unexposed areas in the photographic material, or in other words fogging, and in the liquid, or in other words soiling. It is surprising that even if, owing to these measures, the concentration of the metal salt is materially reduced, the rate of developing generally does not become inadmissibly small and that nevertheless the images become sufficiently black, so that a favourable ratio between the quantity of metal taking part in the production of the image and the waste of metal is ensured. On the contrary, material reduction of the concentration of the reducing agent exerts a detrimental effect both on the rate of developing and on the blackening. The use of a quantity of metal salt slightly in excess of the quantity just sufficient for building up the contrasts has a further advantage in that the metal salt which is usually the most expensive constituent of the physical developer, is utilized as far as possible.

If use is made of physical development according to the invention, little supervision is needed and after development the piled material may be left in the developing liquid for a considerable time. This time may be longer according as the excess of metal salt contained in the developer over the quantity of metal salt which is just sufficient for building up the contrasts is smaller. If this excess is not higher than 100% the time during which the piled material sojourns in the developing liquid is unimportant so long as it is sufficient. A sojourn, for example, for a whole night, even if the development occurs in a considerably shorter period, for example half an hour, is not inconvenient. It is to be noted that in the case of such a long sojourn of the photographic material in the developing liquids fogging or production of stains was never observed, as is the case with chemical development of long duration or of piled quantities of, for example, silver bromide paper. In view of these considerations it is obvious that, according to the invention, use is preferably made of a developing liquid which contains not more than double the quantity of metal salt required for building up the contrasts.

The advantages obtained by using the method according to the invention may therefore be summarized as follows: A great number of sheets of photographic material can be manipulated at the same time, little or no supervision is needed and no costly metal salt is wasted. The contrasts produced were always of satisfactory quality with sufficient blackening and free from fogging and stains.

If the support of the photographic material readily allows the passage of the developing liquid, as in the case, for example with an aqueous developing liquid, of regenerated cellulose and of paper not glued intensely or not glued at all, such, for example, as most kinds of base

paper for phototype, the pile already formed can be put into the developing liquid without inconvenience. Less pervious carrier material, for example heavily glued paper such as writing paper, generally necessitates taking special measures. Thus, for example, the sheets of photographic material may be introduced into the developing liquid one at a time and piled up therein, so that from the start a layer of developing liquid is provided between each pair of consecutive sheets, excellent results being thus obtained. The same result, that is to say sufficiently rapid moistening of the sheets of paper may, however, be obtained by adding to the developer a given quantity of a diffusing agent and for this purpose use may be made with satisfactory result, for example, of the product delivered on sale by the "Imperial Chemical Industries" under the registered trademark of "Lissapol-N". The latter is a wetting agent or detergent which has been described in a paper entitled "Wetting and Detergency" issued in 1937 by the Chemical Society of London and is a polyether as well as a monohydric alcohol having the probable chemical formula:



The quantity required varies with the content of glue in the paper and is generally from some few tenths of a percent to some few percents in the developer. Other diffusing agents are also suitable if they do not result in undue reactions with the developer or the chemicals in the photographic material.

At the moment when the developed pile is removed from the developing bath, the developer is generally exhausted. As already mentioned, it is common practice to use developers having a plentiful proportion of reducing agent compared with their content of metal salt, because such developers yield better results in practice and in addition the reducing agent is almost invariably cheaper than metal salt. Such developers are exhausted as soon as the metal salt is consumed and converted into metal which has served for the formation of the image and may have deposited in part without the photographic material. The remaining solution may still contain a considerable quantity of reducer and may be used to prepare a fresh developer by adding a measured quantity of metal salt, preferably in the form of a concentrated solution. The developer thus regenerated allows of being used again. It should be noted in addition that with the stabilized developers specifically used according to the invention contamination due to oxidation by atmospheric oxygen is of no importance in practice.

The aforesaid stabilized developers may be produced in various ways. A customary physical developer contains 1 or 2% of metol or hydroquinone to which an organic acid, say citric acid or tartaric acid, is added to adjust the pH to approximately 2. This solution provided with, for example, 0.5% of silver nitrate, develops, within a few minutes, a latent image so as to form a silver image and is exhausted in about 10 minutes owing to the metal salt being reduced completely to metal. Such developers allow of being stabilized by diluting them with, say, a 25-fold quantity of water, so that the concentration of the reducing agent has a molarity of not more than 0.01 or by reducing the pH to a value of less than 1, for example of about 0.5, with the use of a strong acid, for example nitric

acid, or else by cooling them, with the addition of glycerol or the like, if necessary, to a temperature lower than 10° C., for example 0° C. or even lower. The time of development thus becomes at least 15 minutes. If care is taken to see that the quantity of metal salt does not appreciably exceed the quantity just required for developing the pile concerned, the pile may be allowed to stand overnight in the developer without objection, without entailing fogging or soiling. After the pile has been removed from the developer, metal salt may again be added to the developing liquid and another pile may be developed therein, as above described.

It often occurs that among the photographic material to be developed there are one or more sheets, or even a whole pile, which are required to be rapidly developed. In accordance with a particular embodiment of the invention, this may be achieved by the photographic material to be rapidly developed, without the pile being subjected sheet by sheet to direct radiation, preferably by infra-red light, and the outer sheet, each time its development is completed, being taken from the pile and removed from the developer. The infra-red rays are substantially absorbed by the sheet on the outside of the pile and more particularly by the image already partially produced.

On the development of the material required to be rapidly developed being completed, any remainder of the pile may be subjected, without radiation, to the action of the developer.

#### Example I

30 foils (size 9 x 12 cms.) of regenerated cellulose were sensitized with a solution of 0.1 n hydroxy-1 diazonium-2 methyl-6 benzene sulphonic acid-4, 0.035 n mercurous nitrate and 0.05 n nitric acid; after drying they were exposed, in contact with a photographic negative, for 30 seconds at a distance of 15 cms. with the use of a high-pressure mercury-vapour discharge lamp of 500 w. The foils were then piled and the pile formed was put into 250 cc. of a dilute physical developer containing 0.05% of metol, 0.01% of tartaric acid and 0.02% of silver nitrate, the prints being left therein for about 6 to 8 hours and being finally washed in water and dried. The contrasts obtained were sharply defined and effective and showed no fogging.

#### Example II

25 sheets of heavily glued paper (size 9 x 12 cms.) were sensitized by immersion in the sensitizing solution referred to in Example I. Subsequent to drying they were exposed, in contact with a photographic negative of a printed text, for 3 seconds at a distance of 25 cms. from a high-pressure mercury-vapour discharge lamp of 500 w. The sheets were then piled in a developing dish containing 125 cc. of dilute physical developer having the following composition: 0.1% of metol, 0.2% of tartaric acid, 0.02% of silver nitrate, everything in water. After 15 minutes or more the pile was removed from the developing dish and the copies were washed and dried. The definition, blackening and effectiveness of all contrasts were satisfactory.

The same result was obtained after a pile had been left standing in the developing liquid overnight.

A similar result was obtained by developing for 15 minutes or more in an equal volume of a di-

lute physical developer containing 0.05% of hydroquinone, 0.02% of silver nitrate. Fogging did not occur.

#### Example III

100 sheets of base paper for phototype (80 grs. per square metre), 9 x 12 cms., sensitized by two-sided application, by rolling, of a solution of 0.4 n hydroxy-1 diazonium-2 methyl-6 benzene sulphonic acid-4, 0.4 n mercurous nitrate and 0.4 n nitric acid, were exposed on both sides in contact with a photographic negative of a printed text, then piled up and introduced all of them at the same time, in the form of a pile, into 250 cc. of a dilute physical developer of the following composition: 0.1% of metol, 0.2% of tartaric acid, 0.04% of silver nitrate, everything in water.

15 After 45 minutes or more the pile was taken out of the liquid. After washing and drying, the copies were found to be of satisfactory quality, whilst a difference between the outermost and the innermost sheets of the pile could not be ascertained.

#### Example IV

25 sheets of base paper for phototype, sensitized in the manner described in Example III and exposed, were combined to form a pile and this pile was immersed, as a whole, in 125 cc. of a strong-acid physical developer containing 1% of metol, 0.3 n nitric acid, 0.02% of silver nitrate, everything in water, and developed. The development of the pile was completed in about 15 minutes and the result was the same as mentioned in the preceding examples, even when the pile was left to stand for a longer period in the developing liquid. When not used, this developer remains stable for a few hours. It may be regenerated by adding 2.5 cc. of a solution of 1% silver nitrate in water.

#### Example V

25 sheets of unglued paper were sensitized in the manner described in Example III dried and unilaterally exposed in the above-mentioned manner. They were combined to form a pile and the pile was immersed in a developer of the composition: 0.1% of metol, 0.2% of tartaric acid, 0.2% of silver nitrate, everything in water.

45 The quantity of developer was 5 cc. per square dm. of paper to be developed.

After a sojourn of 75 minutes in the developer and subsequent to washing and drying of the 50 sheets, the contrasts in all the sheets of the pile were found to be excellent.

#### Example VI

25 sheets of paper, sensitized and exposed in the manner described in Example III were combined to form a pile and immersed, as such, in a developing tank containing 250 cc. of a developer of the following composition: 1% of hydroquinone, 4% of tartaric acid, 25% of glycerol, 0.02% of silver nitrate, everything in water.

60 By cooling this developer was kept at a temperature between -6° and -3° C. After two hours the pile was removed and the sheets were washed and dried. The quality of the contrasts is satisfactory. The sojourn of the pile in the liquid may be prolonged at will. The developer 65 may be regenerated by adding 2.5 cc. of a solution of 1% silver nitrate in water to the exhausted developing liquid. Soiling and fogging 70 do not occur.

This developer may be used to develop at room temperature, the time of development being about 4 minutes. In this case it is necessary for the photographic material to be removed from the liquid at the end of the developing period since the liquid exhibits turbidity of silver and the developer cannot be regenerated by simply adding a fresh supply of silver nitrate.

*Example VII*

25 sheets of base paper for prototype were sensitized and exposed in the manner described in Example III. The sheets were piled up in a developer of the composition mentioned in Example V and this in such manner that a thin liquid layer only covered the pile. After the pile had been standing for 5 minutes in the developer an infra-red radiator ("Philips Helioflux," 500 w.) was ignited at 8 cms. above the liquid surface. After sufficient development, the topmost sheet was removed each time from the pile, washed and dried. After 5 minutes, ten satisfactorily developed sheets were removed from the pile. Without radiation, at least 45 minutes are required for development.

*Example VIII*

20 sheets of heavily glued paper (9 x 12 cms.) were mechanically provided with a solution of the following composition: 0.4 n hydroxy-1 diazonium-2 methyl-6 benzene sulphonic acid-4, 0.4 n mercurous nitrate and 0.4 n nitric acid. They were then dried and exposed in contact with a photographic negative of a printed text for 25 seconds at a distance of 40 cms. from a water-cooled high-pressure mercury-vapour discharge lamp of 500 w. The sheets were put in the form of a pile in a developing dish containing 50 cc. of a developer of the following composition: 0.1% of metol, 0.2% of tartaric acid and 0.02% of silver nitrate in water. After 30 minutes the pile was removed from the developer, after which the sheets were washed in water for 30 minutes and then dried. The outermost sheets of the pile were satisfactorily developed, whereas the innermost sheets, but for the edges, were developed very incompletely only.

On introduction, on the contrary, of a similar pile of 20 sheets of heavily glued paper into 50 cc. of the same developer which contained in addition 4% of the diffusing agent "Lissapol-N" above referred to, it was found that after a lapse of time of 30 minutes all the sheets were developed so as to exhibit satisfactory blackening.

What we claim is:

1. A method of producing photographic metal contrasts which comprises stacking a plurality of sheets of photographic material each of which comprises a lyophilic support carrying a light-sensitive system containing a diazonium compound and a mercurous salt and which has been exposed to light to form a latent photographic contrast thereon in a stable developing liquid containing a metal salt reducible to a metal in solution and a compound capable of reducing the metal salt to a metal, said liquid containing a quantity of said metal salt which is in sufficient amount to completely develop the said latent contrasts in all the sheets but which is less than three times said amount for a time sufficient to completely develop the said latent contrasts.

2. A method of producing photographic metal contrasts which comprises stacking a plurality of sheets of photographic material each of which comprises a lyophilic support carrying a light-

sensitive system containing a diazonium compound and a mercurous salt and which has been exposed to light to form a latent photographic contrast therein, and introducing said stack of sheets into a stable developing liquid containing a metal salt reducible to a metal in solution, a compound capable of reducing the metal salt to a metal, and a diffusing agent, said liquid containing a quantity of said metal salt which is in sufficient amount to completely develop the said latent contrast but less than three times the said amount for a time sufficient to completely develop the said contrasts.

3. A method of producing photographic metal contrasts which comprises stacking a plurality of sheets of photographic material each of which comprises a lyophilic support carrying a light-sensitive system containing a diazonium compound and a mercurous salt and which has been exposed to light to form a latent photographic contrast thereon in a stable developing liquid containing a metal salt reducible to a metal in solution and a compound capable of reducing the metal salt to a metal, said liquid containing a quantity of said metal salt which is in sufficient amount to completely develop the said latent contrasts but less than three times said amount for a time sufficient to completely develop the said latent contrasts, exposing the top sheet of said stack in said solution to infra-red radiation to hasten development of the same, and removing the top sheet to expose the underlying sheet to the infra-red radiation.

4. A method of producing photographic metal contrasts which comprises stacking a plurality of sheets of photographic material each of which comprises a lyophilic support carrying a light-sensitive system containing a diazonium compound and a mercurous salt and which has been exposed to light to form a latent photographic contrast thereon in a stable developing liquid having a pH less than 1 and containing a metal salt reducible to a metal in solution and a compound capable of reducing the metal salt to a metal, said liquid containing a quantity of said metal salt which is in sufficient amount to completely develop the said latent contrasts but less than three times said amount for a time sufficient to completely develop the said latent contrasts.

5. A method of producing photographic metal contrasts which comprises stacking a plurality of sheets of photographic material each of which comprises a lyophilic support carrying a light-sensitive system containing a diazonium compound and a mercurous salt and which has been exposed to light to form a latent photographic contrast thereon in a stable developing liquid containing a metal salt reducible to a metal in solution and less than 0.01 molar amount of a compound capable of reducing the metal salt to a metal, said liquid containing a quantity of said metal salt which is in sufficient amount to completely develop the said latent contrasts but less than three times said amount for a time sufficient to completely develop the said latent contrasts.

6. A method of producing photographic metal contrasts which comprises stacking a plurality of sheets of photographic material each of which comprises a lyophilic support carrying a light-sensitive system containing a diazonium compound and a mercurous salt and which has been exposed to light to form a latent photographic contrast thereon in a stable developing liquid at a temperature lower than 10° C. and containing

a metal salt reducible to a metal in solution and a compound capable of reducing the metal salt to a metal, said liquid containing a quantity of said metal salt which is in sufficient amount to completely develop the said latent contrasts but which is less than three times said amount for a time sufficient to completely develop the said latent contrasts.

ROELOF JAN HENDRIK ALINK.  
CORNELIS JOHANNES DIPPEL  
HARKE JAN HOUTMAN.

## UNITED STATES PATENTS

| Number    | Name    | Date          |
|-----------|---------|---------------|
| 2,067,690 | Alink   | Jan. 12, 1937 |
| 2,138,486 | Fournes | Nov. 29, 1938 |
| 2,183,447 | Dippel  | Dec. 12, 1939 |
| 2,230,977 | Ham     | Feb. 4, 1941  |

## FOREIGN PATENTS

| Number     | Country | Date          |
|------------|---------|---------------|
| 10 369,146 | Germany | Oct. 13, 1920 |
| 814,449    | France  | Mar. 15, 1937 |

## OTHER REFERENCES

15 Clerc, Photography Theory and Practice, published by Sir Isaac Pitman Ltd., New York, N. Y. (1937), pages 268 and 269.

## REFERENCES CITED

The following references are of record in the file of this patent: